

# UNITED STATES PATENT OFFICE.

PETER C. REILLY, OF INDIANAPOLIS, INDIANA.

## PRESERVED WOOD AND METHOD OF MAKING SAME.

No. 901,557.

Specification of Letters Patent.

Patented Oct. 20, 1908.

Application filed February 21, 1907, Serial No. 358,687. Renewed September 16, 1908. Serial No. 453,356.

To all whom it may concern:

Be it known that I, PETER C. REILLY, a citizen of the United States of America, and resident of Indianapolis, in the county of Marion and State of Indiana, have invented certain new and useful Improvements in Preserved Wood and Methods of Making Same, of which the following is a specification.

10 My invention relates to the treatment of wood to preserve it from decay as well as to give greater density and strength by impregnating it with the fluid constituents of tar.

15 The subjects of this invention, therefore, are wood impregnated with a particular compound and a method of rendering wood impervious to the action of water and other destructive influences by impregnating it with a particular compound.

In a companion application, No. 358,686, filed Feb. 21, 1907, I have described the particular compound referred to and its method of preparation. The result of the process 25 there described is a hydro carbon oil, derived by the direct filtration of tar, which is fluid at ordinary temperatures and contains practically all of the oils of the tar, but which is substantially free of solids in suspension. The oils which are contained in the tar, derived from coal, are many; among them is anthracene, which is recognized as one of the best wood preservative materials known to the art. The tar also contains a large 30 quantity of free carbon in suspension. The purpose of the process described in that case is to separate the free carbon from the oils by simple, direct filtration, without the use of any other material, such as petroleum or 35 coal tar spirits, as a solvent for the tar.

Many attempts have been made heretofore to separate the free carbon from tar by thinning the tar with solvents and then filtering, the result of this operation being 45 that a considerable portion of the oils contained in coal tar are precipitated or coagulated by the solvent and are stopped by the filter, so that they are lost to the filtrate. Beside which, the large quantity of solvent 50 spirits necessary to be employed renders the process very expensive and dangerous, because of their inflammable character; and as far as I know, this process has never been employed on a commercial scale. Beside 55 which, it is difficult to recover the spirit

after the operation is completed, so as to use it again.

It has long been known that coal tar was the very best material for the preservation of wood because of its antiseptic and waterproofing quality and the fact that it did not deteriorate in constitution or character under the influence of water or such acids as it would be exposed to in nature, such as exist in salt water and in the ground. Furthermore, it is antiseptic as against insects, but its intractable character and the impossibility of impregnating wood to any considerable depth with this material has prevented its use as a means of preserving wood to an effective extent, although it has been used and is still largely used for superficial coatings.

The reason why tar in its natural state cannot be used for the impregnation of wood 75 is that it contains a large percentage of free carbon, which gives to the material a sticky, viscous character, and which when the tar is applied to the wood even under vacuum or pressure, will stop the pores of the wood and 80 prevent the entrance of the fluid constituents of the tar to any considerable depth.

In my companion application, above referred to, I have described a method by which I can cheaply and easily separate the 85 free carbon from the tar, leaving all the oils of the tar in a state of fluidity, unmixed with free carbon, so that by the use of the ordinary method now employed for impregnating wood I can cause these oils of the tar to 90 penetrate the pores and interstices of the wood and render it waterproof and antiseptic. Beside which, the oils thus derived from tar are insoluble in water, and substantially non-volatile. The proper preservation of wood requires that it shall be made not only antiseptic against animal and vegetable enemies, but that it shall also be made practically impervious to water and air, and that the waterproofing material should 100 permanently fill the pores of the wood and not evaporate at ordinary temperatures, and that it should also extend substantially through the wood, for the reason that when wood is treated and put into service in such forms as paving blocks, piles, or railroad ties, the conditions of service involve an abrasion of the wood to a considerable depth and frequently to an almost complete severance of the wood. It is desirable, therefore,

that the wood should be made permanently waterproof and antiseptic throughout its entire substance. This I have accomplished, and I believe I am the first person who has ever accomplished it in any form and with any material. I believe I am the first who has ever produced a compound which has the property of making the wood antiseptic and waterproof, and which is not volatile, and of forcing that material into and clear through the wood, thus permanently filling all, or practically all of the pores and interstices of the wood with a material which will not evaporate at ordinary temperatures and which will protect it against all of its ordinary enemies and causes of deterioration. In my companion application I have distinguished between the old process of separating free carbon from the oils contained in tar by the use of the words "direct filtration". By these words I desire to be understood as referring to a process by which the free carbon contained in the tar is separated from the oils of the tar without the use of solvents or the admixture of materials which would thin the tar and precipitate or separate any of the oils of the tar; and therefore when I employ the words "direct filtration" in the claims of this application I desire them to have the same meaning.

The method by which my process of impregnating wood is carried into effect is old in the art. It is fully described in Lunge's work on *Coal Tar and Ammonia*, 3rd edition, page 457. The material made and employed by me may be used by other processes for impregnating wood without altering my essential process, which consists of impregnating the wood with the particular material which I have for the first time made or used for that purpose, and the product of this process is wood so impregnated.

In practice I employ a method which consists in heating the wood in either oil or dry steam to a temperature sufficient to vaporize and evaporate the fluids contained in the wood and the removal of the vapors thus formed so as to leave the pores of the wood open and unfilled with fluid or vapor, then filling these pores with the preserving fluid above described by admitting it in a hot

state into a closed vessel containing the wood under vacuum, and then applying pressure upon the fluid in which the wood is submerged, so as to assist its entrance into the pores of the wood. Another old method by which wood may be impregnated is to submerge the wood in hot oil of the particular constitution described above for a period sufficient to cause the evaporation of the contained water and other fluids within the wood, the removal of the vapors thus formed, and then subsequently immersing the wood while still *in vacuo* in cold oil of the same character, with the result that the hot vapor contained in the pores of the wood is at once condensed and the oil enters the pores under atmospheric pressure. Additional pressure may also be applied, if necessary.

It will be understood that my compound derived from coal tar by the separation of free carbon therefrom may be used by mixing with it creosote oil, or chlorid of zinc, or sulfate of copper, or bi-chlorid of mercury, so as to increase its antiseptic character, or the wood may be impregnated with any one or more of these agents and then subsequently treated with my compound without altering or affecting the nature of my invention.

Having thus described my invention, what I claim and desire to secure by Letters Patent is:

1. As a new article of manufacture, wood impregnated with a hydro carbon oil derived by the direct filtration of tar, which oil is fluid at ordinary temperatures, contains practically all of the oils of the tar, and is substantially free of solids in suspension.

2. The process of impregnating wood for the purpose of preserving it from decay, which consists of filling the pores of the wood with a hydro carbon oil derived by the direct filtration of tar, which oil is fluid at ordinary temperatures, contains practically all the oils of the tar and is substantially free of solids in suspension.

Signed by me at New York N. Y. this 9th day of February 1907.

PETER C. REILLY.

Witnesses:

BESSIE E. WASHBURN,  
JAMES GILLIN.